

## UNITED STATES PATENT OFFICE

RENÉ CLAVEL, OF BASEL, SWITZERLAND

## PROCESS FOR WEIGHTING NATURAL SILK

No Drawing. Application filed November 11, 1929, Serial No. 406,527, and in Germany March 16, 1929.

This invention relates to a further modification of the process described and claimed in my prior Patent No. 1,816,959, dated August 4, 1931 for weighing products consisting of natural silk or containing natural silk, in which, as in the main specification, washing, deacidification and neutralization of the material treated with metallic salt solutions, for example stannic chloride, before its introduction into the fixing solution, for example alkali phosphate solution, are omitted and consists in thoroughly centrifuging or squeezing the material after its treatment with metallic salt solution or freezing it in a similar manner from excess of metallic salt solution and then introducing it directly into an acid fixing bath, for example, mono-sodium phosphate solution, to which, if desired, acids or acid salts may also be added. Protective colloids may also be added to the acid fixing bath. In place of mono-sodium phosphate solution di-sodium phosphate solution may also be employed, the alkaline reaction of which has been converted into an acid reaction by the addition of acid substances, for example hydrochloric acid. It is also possible to effect satisfactory spotless weightings without washing the products which have been treated with metallic salt in order to effect hydrolysis.

The invention is illustrated by the following examples:—

1. Skeins of natural silk are dipped for a short time into a bath of stannic chloride of 35° Bé., then lifted out and left for a short time in the air. This operation may be repeated several times. The skeins are then well centrifuged and squeezed out and then, without washing with water, brought for a short time into contact with a 15% solution of mono-sodium phosphate. After the skeins have been wrung out, squeezed out or subjected to suctional filtration and if desired, rinsed for a short time in water, the final treatment of the silk may be effected in a soap-containing water glass bath of at least 1° Bé. at about 40° C.

2. A mixed material, consisting of natural and artificial silk, is dipped into a

bath of stannic chloride of 35° Bé. at room temperature, then withdrawn and left for a short time in the air. This operation may, if desired, be repeated several times. The material is then thoroughly centrifuged and squeezed out and introduced, without previously washing with water, into a 15% mono-sodium phosphate bath, which contains 100 cc. of hydrochloric acid of Sp. Gr. 1.16 per litre. The acid is then neutralized with a 2% cold sodium carbonate solution and the material passed through a 10% di-sodium phosphate solution at 60° C. and then washed. The above treatments are repeated until the material has acquired the desired degree of tin phosphate weighting.

What I claim is:—

1. A process for weighting textiles containing natural silk, comprising the steps of treating the material with a metallic salt solution, freeing it from excess thereof and then introducing it without washing, deacidification or neutralization directly into a bath containing an acid phosphate of a fixed alkali, and finally neutralizing the material.

2. A process for weighting natural silk, comprising the step of treating the material with a metallic salt solution, freeing it from excess thereof and then introducing it without washing, deacidification or neutralization directly into a bath containing an acid phosphate of a fixed alkali, and finally neutralizing the material.

3. A process according to claim 1, wherein in the acid fixing bath comprises a protective colloid.

4. A process according to claim 1, wherein in the acid fixing bath comprises a protective colloid and at least one acid.

5. A process according to claim 1, wherein in the acid fixing bath comprises a protective colloid and at least one acid salt.

6. A process according to claim 1, wherein in the acid fixing bath is a solution of mono-sodium phosphate.

7. A process according to claim 2 wherein in the acid fixing bath is a solution of mono-sodium phosphate.

RENÉ CLAVEL.

55

60

65

70

75

80

85

90

95

100